

## UNITED STATES PATENT OFFICE

2,442,209

## HIGH TEMPERATURE ALLOY

Lee E. Osman, Marblehead, Mass., assignor to  
General Electric Company, a corporation of  
New York

No Drawing. Application May 23, 1945,  
Serial No. 595,486

4 Claims. (Cl. 75—128)

1

The present invention is an alloy adapted for use as a wheel material in supercharger turbines and the like.

It is one of the objects of the invention to provide an alloy which develops sufficient strength from heat treatment without cold working.

In carrying out the present invention I employ an alloy having a carbon content of 0.25 to 0.35%, about 16 to 18% chromium, about 12 to 14% nickel, about 1.75 to 2.25% molybdenum, about 0.8 to 1.2% tungsten, about 0.4 to 0.6% silicon, about 1.25 to 1.75% manganese, about 0.7 to 1.0% columbium, about 0.45% to 1.20% beryllium, with the balance iron. A preferred alloy composition consists of 0.30% carbon, 17% chromium, 13% nickel, 2% molybdenum, 1% tungsten, 0.5% silicon, 1.5% manganese, 0.8% columbium, and 1% beryllium with the balance iron.

The alloy may be forged at 2000—2100° F. to 1600—1700° F. In order to develop the optimum properties in the alloy, it is quenched from a temperature of about 1050° C. and thereafter aged for about 15 to 24 hours at 650° C. The alloy as quenched has a Rockwell C hardness of 15 to 20. After aging at 650° C. the Rockwell C hardness is 40 and remains substantially constant at that figure. The alloy does not air harden.

The structure after solution treating and aging is duplex consisting of a mixture of alpha and gamma solid solutions together with the precipitated compounds and carbides. Precipitated compounds are believed to be complex iron and nickel beryllides. The ratio between the alpha and gamma solid solutions apparently depends on the composition, the nickel-chromium ratio having a decided effect in this respect and also the percentage of beryllium which restricts the gamma field of the iron-nickel-carbon alloys similar to chromium but to a greater extent.

The solution temperature of 1050° C. provides satisfactory results. If a higher solution temperature is employed, for example a solution temperature of about 1150° C. there appears to be a tendency to cause some grain boundary fusion of the beryllium which adversely affects the ductility and also the yield strength and rupture strength of the alloy. The lower solution temperature of 1050° C. avoids this difficulty and also provides material having a higher rupture strength.

Although the maximum hardness in the alloy is obtained with an aging temperature of 500° C., I generally employ an aging temperature of 650° C. since that is usually the maximum operating temperature of supercharger bucket wheels. Above 500° C. the hardness progressively decreases

although no considerable decrease is found up to 700° C. However, at 800° C. a substantial softening takes place.

Tensile and rupture properties at room temperature of my preferred alloy composition in the form of forged bars which have been heated at 1050° C. for one hour, water quenched and aged at 650° C. for 15 hours and then air cooled, are as follows:

| 10 | Bars            | Tested at— | Approximate Proportional Limit | Tensile Strength | Tensile Results |           |
|----|-----------------|------------|--------------------------------|------------------|-----------------|-----------|
|    |                 |            |                                |                  | Elong.          | Red. Area |
| 15 | Radial.....     | Room Temp. | 134, 500                       | 176, 600         | 7               | 6.93      |
|    | Do.....         | 1000° F.   | .....                          | 140, 500         | 10              | 14.18     |
|    | Do.....         | 1200° F.   | .....                          | 117, 000         | 6               | 7.1       |
|    | Do.....         | 1300° F.   | .....                          | 104, 500         | 5.5             | 7.0       |
|    | Do.....         | 1500° F.   | .....                          | 63, 000          | 8.5             | 12.7      |
|    | Tangential..... | Room Temp. | 113, 650                       | 172, 375         | 11.5            | 11.72     |
| 20 | Do.....         | 1200° F.   | .....                          | 114, 200         | 5               | 13.06     |
|    | Do.....         | 1500° F.   | .....                          | 63, 185          | 9.5             | 16.01     |

## Rupture results at 1200° F.

| 25        | Hours | Stress, per sq. in. | Elongation, Per Cent |
|-----------|-------|---------------------|----------------------|
| 100.....  | ..... | 70, 500             | 14                   |
| 1000..... | ..... | 46, 500             | 8                    |

30 Although I prefer to employ an alloy which contains columbium and both molybdenum and tungsten I have employed alloys having approximately the following compositions in which either the columbium or both columbium and tungsten have been omitted:

|    | (1)                                                    | (2)                                                   | (3)                                                     | (4)                                                              |
|----|--------------------------------------------------------|-------------------------------------------------------|---------------------------------------------------------|------------------------------------------------------------------|
| 40 | 0.19% C<br>16.28% Cr<br>11.72% Ni<br>2.0% Mo<br>.90% W | 0.42% C<br>14.9% Cr<br>11.4% Ni<br>3.0% Mo<br>0.95% W | 0.43% C<br>16.15% Cr<br>14.4% Ni<br>2.00% Mo<br>2.51% W | .32-.39% C<br>18.00% Cr<br>13-15% Ni<br>2-2.5% Mo<br>1.1-1.6% Mn |
|    | 1.26% Mn                                               | 1.43% Mn                                              | 1.33% Mn                                                | 1.00% Be                                                         |
|    | 1.04% Si                                               | 0.54% Si                                              | 1.23% Si                                                | .5% Si                                                           |
|    | 1.00% Be                                               | 1.26% V                                               | .64% Be                                                 | Bal. Iron                                                        |
|    | Bal. Iron                                              | 1.00% Be                                              | Bal. Iron                                               | Bal. Iron                                                        |
|    |                                                        | Bal. Iron                                             |                                                         |                                                                  |

45 Given substantially the same heat treatment as my preferred alloy, for example heated to 1150° C., water quenched and aged for about 15 to 24 hours at 650° C., alloys 1, 2, 3 and 4 develop desirable properties without cold working. The optimum properties however are obtained when the alloy contains columbium and both tungsten and molybdenum as indicated in the preferred alloy composition.

50 The alloys containing columbium are specifically claimed in my copending application Serial

No. 784,757, filed November 7, 1947 and assigned to the same assignee as the present invention.

What I claim as new and desire to secure by Letters Patent of the United States, is:

1. A heat treated iron base alloy containing about 0.25 to 0.4% carbon, about 16 to 18% chromium, about 12 to 14% nickel, about 2 to 4.5% metal from the group consisting of tungsten and molybdenum, about 0.4 to 1% silicon, about 1 to 1.75% manganese, about 0.45 to 1.2% beryllium with the balance substantially all iron.

2. A heat treatable iron base alloy containing about 0.25 to 0.35% carbon, about 16 to 18% chromium, about 12 to 14% nickel, about 1.75 to 2.25% molybdenum, about 0.8 to 1.2% tungsten, about 0.4 to 0.6% silicon, about 1.25 to 1.75% manganese, about 0.45 to 1.2% beryllium with the balance substantially all iron.

3. A heat treatable iron base alloy containing about 0.3% carbon, about 17% chromium, about 13% nickel, about 2% molybdenum, about 1%

tungsten, about 0.5% silicon, about 1.5 manganese, about 1.0% beryllium with the balance substantially all iron.

4. A heat treatable iron base alloy containing about .19 to .43% carbon, about 14.9 to 18% chromium, about 11.4 to 15% nickel, .90 to 5.51% of metal from the group consisting of tungsten and molybdenum, about .4 to 1.23% silicon, about 1.1 to 1.75% manganese, about .45 to 1.2% beryllium with the balance substantially all iron.

LEE E. OSMAN.

#### REFERENCES CITED

The following references are of record in the 15 file of this patent:

#### UNITED STATES PATENTS

| Number    | Name         | Date          |
|-----------|--------------|---------------|
| 2,125,929 | Krivobok     | Aug. 9, 1938  |
| 2,161,926 | Jonas        | June 13, 1939 |
| 2,240,064 | Allen et al. | Apr. 29, 1941 |
| 2,373,490 | Mohling      | Apr. 10, 1945 |